

F. E. IVES.  
COLOR PHOTOGRAPHY.  
APPLICATION FILED FEB. 20, 1917.

1,278,667.

Patented Sept. 10, 1918.

Fig. 1.



Fig. 2.



Fig. 3.



Fig. 4.



Fig. 5.



Fig. 6.



Fig. 7



INVENTOR.

BY Frederic E. Ives  
Rogers, Kennedy & Campbell  
ATTORNEYS.

# UNITED STATES PATENT OFFICE.

FREDERIC EUGENE IVES, OF PHILADELPHIA, PENNSYLVANIA.

## COLOR PHOTOGRAPHY.

1,278,667.

Specification of Letters Patent. Patented Sept. 10, 1918.

Application filed February 20, 1917. Serial No. 149,743.

*To all whom it may concern:*

Be it known that I, FREDERIC E. IVES, a citizen of the United States, residing at Philadelphia, in the county of Philadelphia 5 and State of Pennsylvania, have invented certain new and useful Improvements in Color Photography, of which the following is a specification, reference being had therein to the accompanying drawing.

10 This invention relates to the art of color photography, and has more particularly to do with the process or steps involved in the making of a multi-color photograph or picture compounded of blended monocolored images. In its complete aspect the present process may be said to commence with a set of color selection negatives, whether of the two-color or three-color system, or other system, which negatives are producible by 15 well-known methods; and the present invention provides a novel and advantageous mode of proceeding from such negatives to secure the multi-color positives or pictures. In one aspect the present invention may be 20 said to be directed more particularly to the subject of motion pictures in color, a branch of the art of color photography, and in which, on account of the minute size of the images, it has been found difficult to accurately 25 secure or insure exact registration of the component images. The present invention by overcoming such difficulties prevents the incidental formation of fringes of color in the making and exhibiting of color motion pictures.

I will hereinafter for convenience describe the invention as applied to the two-color system, wherein red and green, respectively, may be considered as the selected 30 primary colors, and blue-green and red, respectively, the corresponding secondary or complementary colors. Also, while the invention is applicable to many systems wherein the monochrome components of the positive image are produced successively, the later one being produced directly upon and in registry, so as to blend, with the earlier one, I shall for convenience of description assume the process described in my prior 35 Patent No. 1,170,540 of February 8, 1916, and will point out how the present invention should be practised as an improvement thereon.

In said prior Patent 1,170,540, after obtaining the negatives representing the selected primaries, and which may be respec-

tively referred to as the red-representing negative and the green-representing negative, I proceeded by first making a monochrome positive from one of the negatives. 60 Specifically, I produced a blue-green positive directly from the red-representing negative, this colored positive being carried in a gelatin film on a suitable support. I then used the green-representing negative or a 65 diapositive therefrom to print directly upon the blue-green monochrome print a red image in registry with the blue-green image. This I preferably did by bichromate-sensitizing of the gelatin film containing the 70 blue-green image and then exposing beneath a diapositive from the green-representing negative, and thereafter dyeing the exposed colloid by suitable red dye which is selectively imbibed, forming an image blending 75 with the blue-green image and yielding the desired multi-color print. It will be understood that the negatives and the green-representing diapositive referred to are the usual black, or rather, black and clear, 80 negatives or diapositives. To avoid confusion I shall throughout this specification use the word color or colored in a sense distinguished from black or clear.

In practising the process of Patent 80 1,170,540, I have repeatedly encountered a difficulty which I have now overcome by the present invention. This difficulty was to secure accurate registration of the black green-representing diapositive over the previously 90 formed blue-green monochrome positive. Practically speaking, visual registration is necessary, at least in the first instance, and I have found that the most minute visual examination, however carefully made, has 95 not availed to insure exact registration. The difficulty is enhanced in the case of cinematographic films where the details of the pictures are substantially microscopic, and where, moreover, the slightest inaccuracy in 100 registration is immensely magnified in projecting the picture upon the screen. Inaccuracy in registry means that one or other of the color images, the blue-green or the red, will overlap at various points, thus producing bright color fringes in the projected picture, which is extremely objectionable.

The objects of the present invention are generally to overcome the various defects above mentioned, and particularly to overcome the difficulty in exact registration in 110 the printing or blending of a second mono-

chrome image over a preformed positive print of another color. Other objects and advantages will be explained in the herein-after following description or will be apparent to those skilled in the art.

To the attainment of the above referred to objects and advantages, the present invention consists in the novel process, system, means, products, steps and other features hereinafter described or claimed.

In one aspect the present invention particularly consists in the process of making a blended picture after having secured a preformed color print or positive by photographically printing a differently colored image in registry upon, so as to blend with, the preformed color print by effecting a photographic exposure through a diapositive, or in some cases a negative, which, contrary to the usual black and clear diapositive or negative, is of a color which effectively contrasts with that of the preformed print, so that the eye is easily enabled to effect exact registration before exposing to light to print in the second image. Thereby is overcome the defect in the prior patent that the black and white diapositive affords insufficient contrast with the preformed monochrome image during the step of registration. More specifically, I prefer, after securing the first color image, to use for the printing of the succeeding one a diapositive of the complementary color, so that during the step of registration the observer practically has before him the final multi-color or blended image. Specifically, after securing the blue-green positive in gelatin and resensitizing, I employ a red diapositive secured from the green-representing negative, and with this red diapositive registration above the blue-green image is easily and satisfactorily made prior to the actual exposure and subsequent selective dyeing of the gelatin.

In order to afford a full and complete disclosure of the present invention, and the mode of practising it, I will set forth step by step one practicable mode of procedure and details; and any details not herein fully set forth may be ascertained by reference to said prior Patent 1,170,540, or will be well understood by those skilled in the art; but, since many matters of detail, order of procedure, and other features may be obviously variously modified, I do not intend to limit my invention to the described features excepting in so far as the same may be specified in the claims appended hereto.

In the accompanying drawings illustrative of one application of my invention, Figure 1 in side elevation indicates a red-selection negative, Fig. 2 a green-selection negative, and Fig. 3 a diapositive from the green-selection negative. Fig. 4 indicates the step of printing a blue-green positive on the red-selection, Fig. 5 the step of printing

a red image from the Fig. 3 diapositive in registry upon the blue-green image, and Fig. 6 on an enlarged scale shows the nature of the resulting print. Fig. 7 shows a modification.

70

Commencing the description of the present invention at that point where the color selection negatives have been obtained, and assuming that one of these represents red and the other green, these being the selected primaries, the subsequent procedure may be in detail as follows:

75

Before producing a blue-green positive from the red selection negative 10, it will be convenient to first secure the red diapositive from the green-representing negative 11 for the purpose of using such diapositive in exposing and printing the second of the two monochrome images to be blended.

80

From the black negative 11, which represents green, I print a black diapositive 12, which may be done in a well-known manner, for example, by merely exposing a silver haloid sensitive plate or film beneath the negative and developing in the usual way. I next convert the black diapositive into a red diapositive, and the procedure for this may be as follows:

85

I first soak the diapositive over night in a copper toning solution made up of the following solutions, which can be kept in stock:

90

*Solution A.*

|                       |                  |
|-----------------------|------------------|
| Potassium ferricyanid | 50 grains        |
| Potassium citrate     | 240 grains       |
| Water                 | 100<br>20 ounces |

95

*Solution B.*

|                   |                  |
|-------------------|------------------|
| Copper sulfate    | 60 grains        |
| Potassium citrate | 240 grains       |
| Water             | 105<br>20 ounces |

100

A mixture of equal parts of solutions A and B gives the desired toning solution, and, when the diapositive has been soaked for the requisite time, it will be found to have been converted into a copper red colored image. This image is somewhat degraded by the presence of silver ferricyanid, and I, therefore, prefer to dissolve out this silver salt by the use of sodium thiosulfate ("hypo").

110

I prefer that the diapositive 12 should be of a deeper and brighter red than the copper red so produced, in order to give a more emphatic contrast when registering with the blue-green image, and this result may be accomplished as follows:

120

The copper red diapositive may then be soaked in an aqueous solution of fuchsin dye containing a small quantity of acetic acid. Owing to the fact that copper is a mordant for certain alkali dyes including the one mentioned, the diapositive is caused to take up selectively a substantial amount of the dye. After this treatment the diapositive

130

should be washed out in water containing weak acetic acid, so as to remove the unmordanted part of the dye. The red dia-positive 12 when dry is ready for printing purposes, and it will be understood that it is a green-representing diapositive, colored red to contrast vividly with the blue-green positive monochrome.

The subsequent procedure has already 10 been referred to. The red-representing negative 10 will first be utilized to secure a blue-green positive image, which may be done on the silver conversion system mentioned in Patent 1,170,540, or by any other 15 convenient system. This step is indicated in Fig. 4, in which beneath the negative 10 is seen the print member 13, comprising the sensitive layer 14 over the carrier or glass 15.

Having the blue-green positive image, the 20 second image may be produced and blended in different ways. One well-known procedure would be to first coat the blue-green image with a protective coating of varnish 16, as indicated in Fig. 7, and apply over 25 that a sensitive layer 17 before proceeding to expose and print for the red image. The present invention is independent of the particular location or relative arrangement of the blended images, having to do with the 30 problem of securing registration between the first formed image and the printing member used for printing the second image, which latter I may sometimes indeed locate on the rear or reverse side of the transparent carrier, as has been heretofore proposed. 35 Or I may proceed as in said Patent 1,170,540, wherein the blue-green image is contained in a gelatin layer 14, see Fig. 5, which may now be sensitized with potassium bichromate. 40 This resensitized monochrome may now be exposed beneath the green-representing red-colored diapositive 12. This, as previously explained, is easily and accurately performed by reason of the color contrast 45 between the red diapositive and the blue-green positive image. Following this it is merely necessary to wash out the unaffected bichromate, and immerse for one or two minutes in an acid solution of sodium salt 50 of di-sulfonaphthalene-azo-B-naphthol-disulfonic acid, known as fast red or similar dye. By this procedure the red image will be created by selective absorption and will be 55 found to be accurately registered with the blue-green image, and therefore properly blended, so that, when magnified by projection on a motion picture screen, the objectionable color fringes will be substantially eliminated.

60 In enlarged cross-section the final picture may be somewhat as indicated in Fig. 6, wherein above the transparent carrier 15 the layer 14 of colloid is shown as having embodied in it the blue-green image 18 and the 65 subsequently formed red image 19, the lower

part of the colloid layer being clear, as shown at 20.

In cases where it is desired to use a colored negative as the printing member for the second image, instead of the colored dia-positive, the original black negative may be suitably converted to a red color, for example, in the manner above described; and in this case a different mode of selectively producing the second image will have to be adopted, for example, the use of a dye like eosin, which is mordanted by the chromium compound produced in the film by exposure to light but can be washed out of the unhardened portions, thus producing a red positive image by printing under a negative image.

The particular colors mentioned are only instances, and they may be reversed or suitably altered according to the system of primaries and secondaries that may be selected. In the particular two-color system referred to, the red image may be of various shades of red as circumstances may dictate, and the blue-green image may vary from blue to green, and may, therefore, be referred to as a blue-to-green image.

Other methods than the one given may be employed for converting a black silver image to a colored image, as required for this process. For example, the method of the Traube Patent 1,093,503 of August 14, 1914, wherein the silver image is converted to silver iodid and subsequently dyed with an alkali dye which is mordanted by silver iodid; and a silver image converted to silver ferricyanid will dye selectively with alkali dyes in the same manner. The copper and dye image is preferable for the object of my invention because of its intrinsic color and superior opacity to actinic light, and the greater permanency to light of alkali dyes in combination with the copper mordant. This image, and the process of producing it, have a wider utility than as above described 110 and the same have been divided out from the claims hereof and were made the subject of interference between my divisional application No. 195,508, filed October 9, 1917, and application of J. I. Crabtree No. 115 144,557, filed January 25, 1917, under which respective applications cross-licenses to the owners thereof have been granted.

What I claim as my invention is:

1. In the art of color photography the 120 process of making a multicolor photograph from a set of color selection negatives which represent the respective selected primary colors, said process consisting in printing from one negative a monochrome positive 125 of a secondary color corresponding to the first primary, producing from another negative a colored printing member contrasting in color with such positive, and then printing 130 from said printing member in registry

with said positive a color image of a secondary color corresponding to the second primary.

2. In the art of color photography the process of making a multicolor photograph from a set of color selection negatives which represent the respective selected primary colors, said process consisting in printing from one negative a monochrome positive 10 of a secondary color corresponding to the first primary, producing from another negative a colored diapositive contrasting in color with such positive and then printing from said diapositive in registry with said 15 positive a color image of a secondary color corresponding to the second primary.

3. In the art of color photography the process of making a multicolor photograph from a set of color selection negatives which 20 represent the respective primary colors red and green, said process consisting in printing from the red-representing negative a monochrome positive of a blue-to-green color, producing from the green-representing negative 25 a colored diapositive contrasting in color with such blue-to-green positive, and then printing from said colored diapositive in registry with said positive a red image.

4. In the art of color photography the process of making a multicolor photograph from a set of color selection negatives which represent the respective primary colors red and green, said process consisting in printing from the red-representing negative, a 30 monochrome positive of a blue-to-green color, producing from the green-representing negative a red diapositive, and then printing from said red diapositive in registry with said positive a red image.

40 5. In the art of color photography the process of making a multicolor photograph from a set of color selection negatives which represent the respective primary colors red

and green, said process consisting in printing from the red-representing negative, a 45 monochrome positive of a blue-to-green color and thereafter resensitizing such colored positive, producing from the green-representing negative a color diapositive contrasting in color with such blue-to-green 50 positive, and then printing from said diapositive in registry with said positive a red image.

6. In the art of color photography the process of making a multicolor photograph 55 from a set of color selection negatives which represent the respective primary colors red and green, said process consisting in printing from the red-representing negative a monochrome positive of a blue-to-green 60 color, producing from the green-representing negative a red diapositive by producing a black diapositive and copper-toning it to a red color, and then printing from said diapositive in registry with said positive, a 65 red image.

7. In the art of color-photography the process of making a multicolor photograph from a set of color-selection negatives, consisting in producing a color image by printing from one of the negatives, producing from another of the negatives a diapositive of a color contrasting with the color of the first mentioned image, and subsequently producing in registry with the first image a 75 second image of a different color by printing from said color diapositive.

8. The process of making a multicolored photograph consisting in photographically printing a color image in registry with a 80 preformed color print by exposure through a diapositive having a color that contrasts with the preformed print.

In testimony whereof, I have affixed my signature hereto.

FREDERIC EUGENE IVES.